

## UNITED STATES PATENT OFFICE

DAVID L. LEVY, OF LYNN, MASSACHUSETTS.

## METHOD FOR TREATING HIDES

No Drawing.

Application filed May 20, 1927. Serial No. 193,067.

This invention relates to an improvement in a method or process for treating hides.

The fundamental object is to increase the yield without detriment to the leather, with 5 the ultimate result that the leather is greatly improved.

Heretofore a process has been developed in which the stretched hide fastened to a frame of wood or other material, is submerged in a 10 vat or tank containing tanning liquor of the desired character, where it is permitted to remain until the process of tanning is complete. This process was evidently devised with the intention of increasing the yield by maintaining 15 the stretched condition of the leather during the tanning, and thus preventing shrinkage. For obvious reasons this decreased the quality of the leather, and the practice was otherwise uneconomical and impracticable. 20

With my process, I increase the yield, and at the same time greatly improve the product, and otherwise obviate the objections to the herein referred-to process. In my process, 25 there are three main steps in the procedure:—

Instead of tanning after the hide is stretched, and while in a stretched condition, I first tan it in a vat or tank containing chromium compounds, alum, common salt, 30 and acid, in suitable proportions, for the usual length of time. After this first tanning process, I stretch the leather and fasten it on a frame in the time-honored way.

Then the second step in my process is to prevent the hide (after removal from the frame) 35 from shrinking back to its original or substantially its original proportions; and this is accomplished by putting it through a second tan, adding to the tan liquor a certain amount of common salt varying according to 40 the conditions and nature of the hides being treated.

Following this, the third step is as follows:—While fat-liquoring in the drum 45 heretofore using oil, I add a large percentage of glycerin to the oil in proportions of approximately one part of glycerin to two parts of oil, this being subject to variation according to the nature and condition of the hide. 50 Glycerin nourishes the leather, which is the

desideratum, bringing the fibre closer to the grain, and with the result that while degreasing the hide to make it into patent leather, the oil is removed but the glycerin remains in the leather, as it cannot be extracted. The result is, it gives the product a 55 velvety or silky feel, and at the same time strengthens the leather.

Thus I get the advantage of the increased yield by maintaining the stretched condition 60 without the slightest injury or detriment to the leather, and, on the contrary, produce a greatly improved product.

## I claim:

1. An improved process for treating hides, 65 which consists in first tanning, stretching, and fastening a hide on a frame, then giving it a second tan to which is added a certain amount of salt which varies according to the condition and nature of the hide being 70 treated, with the effect of preventing shrinking of the hide and maintaining its stretched condition, and finally while fat-liquoring in a drum containing oil, adding glycerin, which latter has the effect of nourishing the 75 leather and remaining in it after the oil is removed, thereby strengthening the leather, and at the same time imparting a velvety or silky feel thereto.

2. The process of treating leather including successively tanning it in a vat, stretching it after removal from the vat, tanning it in a liquor containing common salt, and thereafter fat-liquoring it in a drum containing oil and glycerin. 85

3. The process of treating leather including tanning it in a liquor containing common salt, and thereafter fat-liquoring it in a solution containing glycerine.

4. The process of treating leather including tanning the hides and stretching the same, tanning the hides in a liquor containing common salt, and thereafter fat-liquoring them in a solution containing glycerine. 90

In testimony whereof I affix my signature. 95  
DAVID L. LEVY.